

No. 697,831.

Patented Apr. 15, 1902.

H. A. FRASCH.

METHOD OF RECOVERING METALS BY ELECTROLYSIS.

(Application filed Mar. 7, 1901.)

(No Model.)



Fig. 1.



Fig. 2.

Witnesses:

J. M. Long  
A. E. Lamb.

Inventor:

Hans A. Frasch  
by W. H. Finucane  
Atty.

# UNITED STATES PATENT OFFICE.

HANS A. FRASCH, OF HAMILTON, CANADA.

## METHOD OF RECOVERING METALS BY ELECTROLYSIS.

SPECIFICATION forming part of Letters Patent No. 697,831, dated April 15, 1902.

Application filed March 7, 1901. Serial No. 50,254. (No specimens.)

*To all whom it may concern:*

Be it known that I, HANS A. FRASCH, a citizen of the United States, residing at Hamilton, in the county of Wentworth and Province 5 of Ontario, Canada, have invented a certain new and useful Improvement in Methods of Recovering Metals by Electrolysis, of which the following is a full, clear, and exact description.

10 This invention relates to the recovery of metals by electrolyzing an ammoniacal solution of those metals whose hydroxids are soluble in ammonia, and more particularly to the recovery of nickel and copper from ammoniacal solutions.

I am aware that the recovery of metals from ammoniated metallic solutions is old; but in the methods heretofore practiced either insoluble anodes are used or if soluble anodes 20 are used they are composed of the same metal as the one in the electrolyte, and after the metal contained in the solution has been removed there results a solution of sulfate or chlorid of ammonia, according to whatever

25 ammonium salt has been electrolyzed, so that it is necessary to recover the free ammonia from these solutions by distillation in order to allow the electrolyte to be resaturated. To do away with the necessity of this redistillation of the ammonia, I electrolyze the solution of copper or nickel ammonium chlorid or sulfate in presence of a soluble anode, and thereby form at the anode the sulfate or chlorid of the metal of which the anode is com-

30 posed, while the metal contained originally in the electrolyte is deposited upon the cathode, and at the same time the ammonia is set free at the cathode, remaining in solution in free state, so that the same electrolyte can 35 be resaturated with fresh metal and used over again.

I am aware that nickel is deposited by electrolysis from ammoniacal solutions in presence of nickel anodes, and a similar process 45 has been applied to copper; but in this practice the anode has to be composed of the same metal as is contained in the electrolyte, as otherwise the electrolyte would become contaminated with the metals contained in the 50 anode. My invention permits the use of any metal for the anode without contaminating the electrolyte of the cathode, so that, for in-

stance, my anode may consist of copper-nickel matte or ore or other material containing a mixture of iron, copper, nickel, and other metals, 55 and while I deposit nickel from an ammoniacal solution at the cathode I form at the anode the sulfate or chlorid, as the case may be, of all the metals contained in the anode.

To carry out my invention, I prefer to employ the apparatus described in my Patent No. 669,441, dated March 5, 1901; but I do not limit my invention to the use of this or any particular apparatus.

For illustration I will describe my process 65 as carried out in the apparatus above mentioned for the recovery of nickel from nickel-ammonium chlorid as obtained by the invention described in my Patent No. 669,899, dated March 12, 1901.

In the accompanying drawings, illustrating 70 an apparatus which may be employed in carrying out my invention, and in which like parts are correspondingly designated, Figure 1 is a longitudinal section, and Fig. 2 is a top 75 plan view.

For an anode *a* I use copper-nickel matte in comminuted state spread over the bottom of the vessel *b*, conducting the electric current thereto by means of suitable rods or bars 80 *c*, those extending inside of the vessel preferably being of carbon because of its durability. This anode is covered with sand or any other granular electrically and chemically inert substance forming a permeable dia- 85 phragm *d*. The vessel is then filled to the top of the sand with a solution of sodium chlorid, preferably of about 20° Baumé in strength. The remaining space of the vessel above the diaphragm is supplied with a solution of 90 nickel-ammonium chlorid containing an excess of ammonia, or I may use a solution of the normal nickel-ammonium chlorid, adding thereto free ammonia until the latter is in excess. The cathodes *e* are suspended above 95 the diaphragm, and they may consist of any suitable metal, in this instance preferably nickel, and the whole is then subjected to an electric current of proper density. The nickel thereby is precipitated in metallic form upon the cathodes, while the chlorin in chemical combination with the ammonia and nickel is liberated at the anode, there forming the chlorids of copper, nickel, iron, and whatever

metals are contained in the anode. This chlorid solution may be continuously or periodically removed from the anode-section of the apparatus below the diaphragm by dis-  
 5 placement with fresh solution of sodium chlo-  
 rid or any other solvent supplied through pipe  
 f. The ammonia liberated at the cathode by  
 the removal of the chlorin remains in solu-  
 10 tion in the cathode electrolyte, and electroly-  
 sis may be conducted until the last trace of  
 nickel has been removed from the cathode  
 electrolyte, so that only a solution of free  
 15 ammonia remains, which can then be used  
 over again for the production of fresh nickel-  
 ammonium chlorid without the necessity of  
 distillation. Circulation of the electrolyte  
 20 may be secured by means of pipes f and g  
 and the interposed siphon, pump, or other ap-  
 paratus h.

20 In applying the process the cathode elec-  
 trolyte, consisting of a solution of an am-  
 monium double salt bearing the metal to be  
 deposited, is circulated above the diaphragm  
 25 d by means of the pipes g, the anode-section  
 below the diaphragm having been first sup-  
 plied with a solution of sodium chlorid. The  
 electric current being passed between the  
 30 cathode and the anode, the metal contained in  
 the cathode electrolyte is deposited upon the  
 cathode, while the halogen or acid radical  
 contained in the cathode electrolyte is trans-  
 35 ferred to and chemically bound by the metals  
 represented in the anode, forming the corre-  
 sponding metal salts. The salt brine in the  
 anode - section dissolves the metallic salts  
 40 formed there and is then displaced by a fresh  
 supply of salt brine introduced through pipe  
 f at one end, the concentrated metallic solu-  
 tion being drawn off through a similar pipe  
 45 at the other end. The circulation of the two  
 electrolytes above and below the diaphragm  
 may be continuous or periodical. I prefer to  
 maintain a continuous circulation through the  
 50 cathode-compartment, removing the metallic  
 solution from the anode-compartment period-  
 45 ically whenever it has reached any desired de-  
 gree of concentration. Thus I may subject an  
 electrolyte consisting of a solution of nickel-  
 ammonium chlorid in the cathode-compart-  
 55 ment to an electric current, the anode-compart-  
 ment being charged with zinc ore, and  
 deposit metallic nickel upon the cathode, while  
 simultaneously producing a solution of zinc  
 chlorid in the anode without contaminating  
 either of the electrolytes with the metals con-  
 tained in the other.

What I claim is—

1. The process of recovering metals by elec-  
 trolysis, which consists in electrolyzing a dou-  
 ble salt of ammonia and metals whose hy-  
 droxids are soluble in ammonia, in presence  
 of a soluble anode and an anode electrolyte  
 (anolyte) containing metals different from the  
 one contained in the cathode electrolyte (cath-  
 olyte) but free from ammonia.
2. The method of electrolyzing a double salt  
 of ammonia and metals whose hydroxids are

soluble in ammonia, consisting of electrolyz-  
 ing a solution of an ammonium double salt  
 containing metal in presence of an anode ca-  
 pable of combining with the acid or halogen  
 radicals contained in the ammonium double  
 salt, and having constituents different from  
 the contents of the electrolyte.

3. The method of recovering ammonia from  
 an electrolyte composed of an ammonium dou-  
 ble salt, consisting in electrolyzing a solution  
 of an ammonium double salt containing metal  
 in presence of a suitable cathode, and an  
 anode capable of binding the acid or halogen  
 radical of the ammonium salt, the cathode  
 and anode being separated by a suitable dia-  
 phragm, depositing the metal contained in  
 the solution upon the cathode, and binding  
 the acid or halogen radical to the substance  
 of the anode, keeping the ammonia in solu-  
 tion in the cathode electrolyte.

4. The method of recovering nickel from a  
 nickel-ammonium salt, consisting in supply-  
 ing an electrolytic bath with an anode com-  
 posed of a metal-bearing substance in com-  
 minuted form, covering it with a chemically  
 and electrically inert permeable substance  
 above which suitable cathodes are arranged,  
 supplying the anode with a solution capable  
 of dissolving the metallic salts there formed,  
 supplying the cathode with a solution of the  
 nickel-ammonium salt, subjecting it to an elec-  
 tric current, depositing the nickel upon the  
 cathodes, and displacing the metallic solution  
 at the anode by a fresh supply of solvent, keep-  
 ing the ammonia in solution in the cathode  
 electrolyte.

5. The process of recovering nickel by elec-  
 trolysis, which consists in supplying a cathode  
 with a solution of nickel-ammonium chlorid  
 containing an excess of ammonia, and sup-  
 plying a soluble anode consisting of different  
 metals with a solution of sodium chlorid, sepa-  
 rating the two solutions by means of a per-  
 meable diaphragm, and by means of an elec-  
 tric current precipitating the nickel in me-  
 tallic form upon the cathode, and forming at  
 the anode a solution of the chlorids of the va-  
 rious metals contained in the anode, substan-  
 tially as described.

6. The process of recovering nickel by elec-  
 trolysis, which consists in supplying a cath-  
 ode with a solution of nickel-ammonium chlo-  
 rid containing an excess of ammonia, and sup-  
 plying a soluble anode consisting of dif-  
 ferent metals with a solution of sodium chlo-  
 rid, separating the two solutions by means of  
 a horizontal permeable diaphragm, and by  
 means of an electric current precipitating the  
 nickel in metallic form upon the cathode,  
 forming at the anode a solution of the chlo-  
 rids of the various metals contained in the  
 anode, and displacing the chlorid solution  
 from below the diaphragm by addition of  
 fresh sodium-chlorid solution.

7. The process of recovering nickel by elec-  
 trolysis, which consists in supplying a cath-  
 ode with a solution of nickel-ammonium chlo-

rid containing an excess of ammonia, and supplying a soluble anode consisting of different metals with a solution of sodium chlorid, separating the two solutions by means of a horizontal permeable diaphragm, and by means of an electric current precipitating the nickel in metallic form upon the cathode, forming at the anode a solution of the chlorids of the various metals contained in the anode, 10 placing the chlorid solution from below the diaphragm by addition of fresh sodium-chlorid solution, and further electrolyzing the cathode solution until the last trace of nickel has been removed.

15 8. The process of recovering nickel by electrolysis, which consists in supplying a cathode with a solution of nickel-ammonium chlorid containing an excess of ammonia, and supplying a soluble anode consisting of different 20 metals with a solution of sodium chlorid, sep-

arating the two solutions by means of a horizontal permeable diaphragm, and by means of an electric current precipitating the nickel in metallic form upon the cathode, forming at the anode a solution of the chlorids of the various metals contained in the anode, 25 displacing the chlorid solution from below the diaphragm by addition of fresh sodium-chlorid solution, and further electrolyzing the cathode solution until the last trace of nickel 30 has been removed from the cathode electrolyte, and utilizing the remaining solution of free ammonia for the production of fresh nickel-ammonium chlorid.

In testimony whereof I have hereunto set 35 my hand this 25th day of February, A. D. 1901.

HANS A. FRASCH.

Witnesses:

WILLIAM E. WOODRUFF,  
W. J. DEVINE.